

F. GIOLITTI.

CEMENTATION PROCESS FOR ARMOR PLATES EMPLOYING MIXED CEMENTATION AGENTS.  
APPLICATION FILED OCT. 14, 1914.

1,195,459.

Patented Aug. 22, 1916.

Fig. 1



Fig. 2



Fig. 3



Witnesses:-

Charles B. Crompton  
May G. Guttrall

F. Giolitti  
Inventor.

By *Eugene D. Marks*  
Attorney.

# UNITED STATES PATENT OFFICE.

FEDERICO GIOLITTI, OF TURIN, ITALY, ASSIGNOR TO SOCIETÀ ANONIMA ITALIANA  
GIO ANSALDO & C., OF GENOA, ITALY.

## CEMENTATION PROCESS FOR ARMOR-PLATES EMPLOYING MIXED CEMENTATION AGENTS.

1,195,459.

Specification of Letters Patent. Patented Aug. 22, 1916.

Application filed October 14, 1914. Serial No. 866,701.

*To all whom it may concern:*

Be it known that I, FEDERICO GIOLITTI, a subject of the King of Italy, and residing at 75 Stradale Moncalieri, Turin, Italy, have 5 invented a certain new and useful Improved Cementation Process for Armor-Plates Employing Mixed Cementation Agents, of which the following is a specification.

The object of the invention is to provide 10 an improved process for the cementation of armor plates by employing together solid and gaseous cementation agents, wherein the undesirable results arising from the exposure of the pipe conveying the gaseous cementation agent to the action of the heated furnace gases are avoided and the gaseous reagent is more uniformly distributed over the surface to be treated and thus the cementation is effected with a greater degree of 15 uniformity.

A further object of the invention is to facilitate the replacement of the solid cementation agent which is consumed in the process and thus further to assist in obtaining 20 a more uniform cementation effect.

According to the invention the armor plates are vertically disposed upon the hearth of the cementation furnace and coupled together by means of metallic prisms or 25 sheets, in such a manner as to form with the faces to be cemented the larger walls of a flat box supported by the hearth at one of its open sides. This lower open side serves for introducing the cementing gas, while the 30 upper open side serves for introducing the solid cementation agent consumed during the process.

The invention is illustrated by way of examples in the accompanying drawings 35 wherein,

Figure 1 shows in a horizontal section two armor plates placed in an ordinary gas fired furnace having a movable hearth. Fig. 2 is a vertical section of the same. Fig. 3 shows 40 in a vertical section the same arrangement applied in a double fired gas furnace having a movable hearth.

The same letters denote like parts in all the figures.

50 A, A', A'' and A''' represent armor plates set on edge, B represents a prism and B' a plate employed for connecting the two plates

together thus forming with the armor plates a hollow prism on the upper end of which is mounted a refractory box C, C, C. A gas 55 conduit D provided with nozzles is arranged in the movable hearth E upon which the armor plates are mounted. The box-like space formed by the plates A, A', or A'', A''', is filled with a solid cementation agent, 60 for instance, carbonaceous material F.

G, G, are wheels on which the movable hearth runs.

H, H, are inner walls of the furnace, the outer walls of which are indicated by K. 65 The fire gases pass into the furnace chamber by the openings L and the waste gases pass out at M, while the gaseous cementation agent is introduced by way of the pipe D which traverses the movable hearth E. 70

The furnace illustrated in Fig. 3 is provided with two movable hearths, the furnace gases passing into the furnace at each side and out by way of a central flue by which arrangement a better utilization of the furnace and a more uniform heating of the plates is attained. 75

The purpose of the box C, C, C. is to provide a container for a reserve of the solid cementation agent to replace that introduced 80 between the plates and which during the process becomes consumed.

Having now described my invention, what I claim as new and desire to secure by Letters Patent is:—

1. A process for cementing armor plates comprising arranging the plates vertically on the hearth of a furnace, filling the space intervening between the plates with a solid cementation agent and introducing a gaseous 90 cementation agent through the hearth of the furnace into the space between the plates.

2. A process for cementing armor plates comprising arranging the plates vertically on the hearth of a furnace, connecting together the plates by means of metal plates or prisms, filling the box-like space thus formed with a solid cementation agent and introducing a current of a gaseous cementation agent through the hearth of the furnace 100 into the space thus formed.

3. A process for cementing armor plates comprising arranging the plates vertically on the hearth of a furnace, arranging a re-

fractory box on the upper edges of the plates, filling the box and the space between the plates with a solid cementation agent, and introducing a gaseous cementation agent 5 through the hearth of the furnace into space between the plates.

In testimony whereof I have signed my

name to this specification in the presence of two subscribing witnesses.

FEDERICO GIOLITTI. 10

Witnesses:

GIACOMO CARDARO,  
A. BORNQUIS GAURA.